

# United States Patent [19]

Muckelroy

[11] 3,812,442

[45] May 21, 1974

[54] CERAMIC INDUCTOR

[76] Inventor: William L. Muckelroy, P.O. Box 9685, Washington, D.C. 20016

[22] Filed: Feb. 29, 1972

[21] Appl. No.: 230,247

[52] U.S. Cl. 336/83, 29/602, 336/192, 336/200, 336/232

[51] Int. Cl. H01f 17/06

[58] Field of Search 336/83, 200, 232, 221, 336/192; 340/174 CC, 174 JA; 317/258; 174/68.5; 338/308

[56] References Cited

UNITED STATES PATENTS

|           |         |                     |            |
|-----------|---------|---------------------|------------|
| 3,483,499 | 12/1969 | Lugten              | 336/200 X  |
| 2,629,860 | 2/1953  | Chesus et al.       | 336/200 X  |
| 3,247,573 | 4/1966  | Loack               | 336/200    |
| 3,665,267 | 5/1972  | Acello              | 317/258    |
| 3,518,756 | 7/1970  | Bennett et al.      | 336/200 X  |
| 2,557,983 | 6/1951  | Linder              | 174/685    |
| 3,400,455 | 9/1968  | Cosgrove            | 340/174 CC |
| 3,058,078 | 10/1962 | Hoh                 | 336/83 X   |
| 3,554,797 | 1/1971  | Coerver, Jr. et al. | 336/83     |
| 2,966,704 | 1/1961  | O'Brian et al.      | 336/221 X  |

|           |         |                 |            |
|-----------|---------|-----------------|------------|
| 3,319,207 | 5/1967  | Davis           | 336/221 X  |
| 3,040,301 | 6/1962  | Howatt et al.   | 340/174 CC |
| 3,282,730 | 11/1966 | Johnston et al. | 338/308 X  |

FOREIGN PATENTS OR APPLICATIONS

993,265 5/1965 Great Britain 336/200

Primary Examiner—Thomas J. Kozma  
Attorney, Agent, or Firm—Edward J. Kelly; Herbert Berl; Saul Elbaum

[57]

ABSTRACT

A nonolithic microminiature inductor comprising a helical conductive path of deposited metal film immersed in a rectangular block of magnetic refractory material. The inductor has metal caps at each end of the block as terminations. These terminations may be soldered to metallized pads located on a substrate. A method for making this inductor wherein loops of conductive metal are deposited onto a thin unsintered magnetically permeable ceramic sheet with holes for interconnection therein and wherein said holes are aligned and said sheets are laminated such that upon sintering said metal forms a helical contiguous conductive path immersed a contiguous block of ceramic.

3 Claims, 19 Drawing Figures



SHEET 1 OF 6

FIG. 1a



FIG. 1b



SHEET 2 OF 6

FIG. 2a



FIG. 2b



FIG. 3a



FIG. 6a



FIG. 6b



PATENTED MAY 21 1974

3,812,442

SHEET 4 OF 6



FIG. 3c



FIG. 3e



SHEET 5 OF 6

FIG. 4



PATENTED MAY 21 1974

3,812,442

SHEET 6 OF 6



## CERAMIC INDUCTOR

## RIGHTS OF THE GOVERNMENT

The invention described herein may be manufactured, used, and licensed for or by the United States Government for governmental purposes without the payment to the inventor of any royalty thereon.

## BACKGROUND OF THE INVENTION

This invention relates generally to monolithic micro-miniature components for use in the assembly of micro-circuitry using substrates as a basis onto which the various types of components are mounted. Less generally this invention relates to a monolithic microminiature inductance element and a method for making same. Specifically this invention relates to a microminiature monolithic inductance element with a magnetically permeable core comprising a magnetically loaded ceramic material and a process for making in mass production large quantities of this device at very economical prices. Moreover, it is related to that class of devices classified as inductors which possess an innercore having the property of significantly enhancing a magnetic field. Among the classes of microelectronic manufacture to which this invention applies are thick film technology, thin film technology, and hybrid multichip technology. In any case, the invention is to be used where reduction in size is required; a large quantity is to be produced; and cost is an essential factor.

Currently spiral inductors made by the application of thick and thin films and by subtractively etching the inductor are currently used in manufacturing hybrid microelectronic circuits. Helical miniature inductors have been available for sometime in monolithic form factors having iron cores. However, they comprise fine wire, wound onto iron rods, coated with an epoxy in order to fix the position of the wire to maintain the characteristics of the device. Many problems exist with such a structure, one of which is a possibility of the epoxy breaking down or a particular piece of wire becoming loose. Such flaws in this type of device under abnormal physical condition can cause severe changes in circuit characteristics. This is especially true in military applications where hardware comprising electronic circuitry is subjected to large accelerations and shocks.

There are other designs of monolithic inductors essentially the same as the one previously described. The difference is that these other devices are molded into plastic. And naturally, there are the myriad of structures for inductive elements which are not microminiature and which are not monolithic in the sense of this invention in that the various parts of the inductor are not chemically bonded or thermally fused to each other. In general, in the past inductors in microminiature form-factors and form-factors easily applicable to hybrid microelectronic circuits have been extremely expensive in relationship to the cost of other functional components to be used in the circuits and therefore offers a cost factor against the use of such components.

Another inherent disadvantage in the structure of the aforesaid components is the nature of the conductive terminations formed onto the device for interconnecting them into the particular circuitry for which it is needed. In most cases, such as that of the plastic device it is best to only epoxy such a device to the substrate using a conductive epoxy material because of the prob-

lems involved in raising the temperature of such a device to that necessary for soldering into the circuit. The difference in thermal coefficients between the plastic and the metal terminations at the ends thereof usually precludes the use of high or even moderate soldering temperatures for interconnecting such devices into the circuit. These differences in thermal coefficients are extremely cumbersome when soldering microminiature devices. In general, in assembling hybrid circuits it is desirable to reflow solder chips components. This precludes other sensitive semiconductors from having to be reheating many times. All devices in use today, except spiral depositions onto substrates, have significant thermal mismatches in materials.

In the case of the spiral inductor printed onto a substrate such as alumina or mylar the coupling between the various turns of the spiral are not enhanced significantly. Usually there is free space above the spiral unless some particular type of coating is applied.

One problem with spiral inductors printed on very thin sheets of material is the high probability of changes in the Q-factor by bending of the substrate. Another problem with the spiral is interconnection. When both terminations of the spiral are on the same side of the substrate one of the terminations must be crossed over the respective turns of the spiral. This degrades operation of the device. Even if terminations are brought out on opposite sides of the substrate the problem of traversing the respective windings is still present. Another severe problem with the spiral inductor and the spiral inductor reversed upon itself is that a tremendously large amount of substrate is required.

The term "refractory material" is used herein to mean a substance which will not melt, decompose or materially change under the processing conditions involving in forming the device herein described. Refractory material is generally classified into four broad groups. The group of utility here includes the polycrystalline materials such as ceramics and includes, for example, porcelains, steatites, aluminas, and ferrites. The present invention is described with reference to these ceramics and, more particularly, thin sheets of alumina with ferrites mixed therein. However, it should be understood that the present invention is equally applicable to the other ceramic materials.

The spiral may be formed from a paste of glass, high melting point metal such as platinum and gold, and a decomposable fluid suspending agent applied to the refractory oxide by any convenient method, for example, by dipping, brushing, or spraying. The relative amounts of materials within the paste may vary over fairly wide limits. The main consideration is that the metal content be sufficiently high to insure that the resulting metal film after processing is continuous. The amount of fluid used as a suspending agent depends on the method of application. If spraying is used, a relatively thin suspension is required. If brushing or "squeeze" screen processes are employed, thicker paste suspension should be such as to insure good conductivity of the deposition.

Magnetic materials usable for this device include 2-81 permalloy and carbonyl iron insulated powders, and Ferroxcube III sintered powder.

Generally, a mean particle size range which is suitable is 0.5 to 25 microns for the paste, with the preferred range being between 0.5 and 15 microns. Smaller particles are equally satisfactory.

As for the glass flux, a glass which fuses and bonds to the ceramic at a temperature below the melting point of the metal and resists reduction under the usual processing conditions should be used.

Glasses having these properties are readily compounded from mixtures of silica ( $SiO_2$ ) and various combination of the oxides of sodium ( $Na_2O$ ), calcium ( $CaO$ ), barium ( $BaO$ ), magnesium ( $MgO$ ), aluminum ( $Al_2O_3$ ), boron ( $B_2O_3$ ), potassium ( $K_2O$ ) and phosphorus ( $P_2O_5$ ), among other elements. Table I is illustrative of some suitable glasses which can be conveniently compounded from typical oxides specified as to kind and amount in the table. The table is not intended to be exhaustive of suitable glasses but indicates the general composition of some readily fusible nonreducible glasses. It is noted that this table encompasses many common types of glasses such as the borosilicates, phosphates and silicates.

TABLE I

| Melt Ingredient: | Parts by Weight |
|------------------|-----------------|
| $Li_2O$          | 0-15            |
| $Na_2O$          | 0-25            |
| $CaO$            | 0-10            |
| $BaO$            | 0-20            |
| $MgO$            | 0-2             |
| $Al_2O_3$        | 0-35            |
| $SiO_2$          | 5-80            |
| $B_2O_3$         | 0-30            |
| $K_2O$           | 0-5             |
| $P_2O_5$         | 0-80            |

In the preparation of the glasses, the ingredients are smelted together in a furnace at a temperature sufficient to melt but not volatilize the constituent oxides, for example, between 1,100° and 1,500° C, until a mass of uniform quality has been obtained. The melt is fritted by pouring into cold water, and the resultant frit is ground to the fineness desired. It is desirable for the glass particles to be finely divided, for example, in the order of  $\frac{1}{2}$  micron to 25 microns particle size, so that the paste mixture will, under the processing conditions, result in a continuous metal layer adherently bonded to the ceramic.

The glass and metal particles are suspended in a volatile and decomposable fluid suspending agent and applied to the refractory oxide by any of the methods aforementioned. The relative amount of metal and glass used may vary over fairly wide limits. The main consideration is that the metal content be sufficiently high to insure that the resulting metal film after processing is continuous. Generally, between five to 50 parts by weight of metal is used for each part by weight of glass.

The fluid suspending medium serves to disperse the paste mixture in the desired pattern on the substrate and to hold the paste in this pattern until processing commences. During processing the suspending medium should volatilize, leaving no residue. The suspending medium should not react with the metallic or glass components of the coating composition before or during firing.

To insure proper dispersion and bonding of the paste, many of the common suspending media contain two components. The first component acts as a dispersion medium for the paste and as a solvent for the second component which insures proper bonding of the paste to the "green ceramic" or refractory oxide until processing commences. Examples of suitable dispersion media which are solvents for the below listed binders

are benzene; the esters of fatty acids; alcohols of low molecular weight such as ethyl, butyl, and amyl; acetates including "Cellosolve acetate" (ethylene glycol monoethyl ether acetate), and "Carbitol acetate" (diethylene glycol monoethyl ether acetate); ketones such as acetone and methyl-ethyl-ketone; and higher ethers such as glycol diethyl ether. Suitable binders are, for example, the vinyl or substituted vinyl polymers such as polymethylmethacrylate, polyethylmethacrylate, polybutylmethacrylate, and polyisobutylmethacrylate and the cellulose esters and ethers such as cellulose nitrate, cellulose acetate, cellulose butyrate, methyl cellulose and ethyl cellulose. Rohm and Haas "Acryloid A-10," a solution of 30 percent polymethylmethacrylate solids in "Cellosolve acetate" has proved a good suspending medium.

In general, any ceramic which is resistant to the usual processing conditions may be used as the refractory substrate. The following table is illustrative of various ceramic compositions that have successfully been used. The compositions are expressed in parts by weight.

TABLE II

| Composition     | Porcelain |    |    |    | Steatite | Alumina       |
|-----------------|-----------|----|----|----|----------|---------------|
|                 | A         | B  | C  | D  |          |               |
| Feldspar.....   | 35        | 50 | 30 | 25 |          |               |
| Ball clay.....  | 15        | 10 | 8  | 10 |          |               |
| Kaolin.....     | 30        | 30 | 37 | 40 | 15       |               |
| Talc.....       |           |    |    |    | 60       |               |
| Dolomite.....   |           |    |    | 2  |          |               |
| $BaCO_3$ .....  |           |    |    |    | 17.5     |               |
| $MgCO_3$ .....  |           |    | 1  |    | 7.5      |               |
| $SiO_2$ .....   | 20        | 10 | 25 | 22 | 9-10     | 2             |
| $CaO$ .....     |           |    |    |    | 1        | 1             |
| $MgO$ .....     |           |    |    |    | 3-4      | 1             |
| $Na_2O$ .....   |           |    |    |    | 1-5      | $\frac{1}{2}$ |
| $Al_2O_3$ ..... |           |    |    |    | (1)      | 95.5          |

<sup>1</sup> Remainder.

In order to form a ceramic slurry with good flow property, the forementioned thermoplastic organics are used as flow-promoting binders for the refractory oxide. The prime step is to coat the fine alumina particles with these thermoplastics. This step is facilitated by intense mixing at high temperatures in the range 100° to 400° C. Water emulsions of the organic plastic agents facilitate the initial mixing of the organic with the ceramic particulates, and the initial contact can be made by using an aqueous or non-aqueous slurry and solution. Removal of the volatile constituents provides an intimate mixture of the organic and ceramic most often termed "green ceramic."

In a typical process, firing of the laminate is done in a furnace in which both atmosphere and temperature can be controlled. The firing is done in an reducing atmosphere. This firing step is carried out under conditions sufficient to volatilize the fluid suspending media, and to commence formation of a refractory ceramic-to-glass-to-metal bond. The temperature and firing times are interdependent. The fluid suspending vehicle used and the temperature required commences formation of the refractory ceramic-to-glass-to-metal bond. This temperature is dependent upon the temperature re-

quired to sinter the ceramic and to cause wetting of the refractory ceramic and at least part of the metal by the glass in the paste system. Such wetting and sintering temperatures are dependent upon the glass flux used. Temperatures ranging from, for example, 1,400° to 1,600° C have been successfully used.

The maximum temperature is limited by the melting point of the metal while the minimum temperature is again dependent upon the wetting and sintering temperature of the glass flux employed and the temperature required to sinter the ceramic wet by the glass comprising the paste.

The invention described herein overcomes many of the disadvantages of the foregoing constructions.

It is therefore the object of this invention to provide a new and novel process for manufacturing microminiature monolithic inductance elements with a magnetically permeable core.

It is yet another object of this invention to provide a new and novel microminiature inductance element with a magnetically permeable core which is monolithic and comprises materials having coherent thermal coefficients.

It is yet an additional object of this invention to provide a new and novel device and process for manufacturing said device which is economical and easily adaptable to high volume manufacturing.

It is yet an additional object of this invention to provide a monolithic helical inductor emersed in a magnetically permeable ceramic material within terminations suitable for attachment by reflow soldering to thick film circuitry.

It is another object of this invention to provide a microminiature monolithic inductance element which has a form factor compatible with that of other components used in hybrid microelectronics.

It is still additional object of this invention to provide a microminiature monolithic inductance element with a structure made of ceramic and cermet materials.

It is yet another additional object of this invention to provide an inductance device having a surface of refractory material.

It is yet an additional object of this invention to provide a microminiature monolithic inductor with a new and novel core comprising a magnetically permeable alumina ceramic.

It is yet an additional object of this invention to provide a helical inductor imbedded in a magnetically permeable alumina ceramic having a rectangular-solid form-factor.

Yet another additional object of this invention is to provide a new and novel microminiature monolithic inductor whose electrical paths are formed by metalization paths of thick films and thin films.

Still an additional object of this invention is to provide a new and novel method for making a microminiature monolithic inductor in which the electrical conductive paths are formed onto unfired alumina ceramic tape by a subtractive etching technique.

Still yet an additional object of this invention is to provide a new and novel design of metalization which provides a helical spiral that provides inductivity within a compact area.

These and other objects of the present invention will become more fully apparent with the reference to the following specifications and drawings which relate to

several variations of a preferred embodiment of the invention described herein.

#### SUMMARY

A monolithic microminiature inductor comprising a helical conductive path of deposited metal film immersed in a rectangular block of magnetic refractory material. The inductor has metal caps at each end of the block as terminations. These terminations may be soldered to metallized pads located on a substrate. A method for making this inductor wherein loops of conductive metal are deposited onto a thin unsintered magnetically permeable ceramic sheet with holes for interconnection therein and wherein said holes are aligned and said sheets are laminated such that upon sintering said metal forms a helical contiguous conductive path immersed a contiguous block of ceramic.

#### BRIEF DESCRIPTION OF THE DRAWINGS

20 The specific nature of the invention as well as other objects, aspects, uses, and advantages thereof will clearly appear from the following description and from the accompanying drawings, in which:

FIG. 1a is an illustration of the process of manufacturing magnetically permeable ceramic tape.

FIG. 1b is a flow chart of the method for manufacturing magnetically permeable ceramic tape.

FIG. 2a is an illustration of the pattern deposition process by which conductive paths are formed on the 30 ceramic tape.

FIG. 3a is a view of the underside and top of various layers of the inductor.

FIG. 3b is an exploded view of a monolithic inductor and unbent metal end terminations.

35 FIG. 3c is an illustration of a monolithic inductor with end terminations about to be bonded thereto.

FIG. 3d is an illustration of a monolithic inductor having end terminations formed by coating the ends thereof.

40 FIG. 3e is an illustration of a finished monolithic inductor.

FIG. 3f is an illustration of a monolithic inductor having its coated end terminations sintered.

FIG. 4 is a flow chart of the manufacturing process 45 by subtractive etching.

FIG. 5a is an exploded view of the monolithic inductor showing internal structure.

FIG. 5b is an illustration of a molded metal end termination or cap.

50 FIG. 5c is an illustration showing a metal end cap with metal film formed thereon.

FIG. 5d shows details of a first outside layer of the monolithic inductor.

FIG. 5e shows details of an interconnector pattern formed on an internal layer of the monolithic inductor.

55 FIG. 5f shows details of a second outside layer of the monolithic inductor.

60 FIG. 6a is an illustration of two adjacent layers of ceramic tape with conductive patterns thereon before lamination.

FIG. 6b is an illustration of two adjacent layers laminated with the interconnection of the conductive metalization from one layer to the next.

65 These and other objects of the present invention will become more fully apparent with reference to the following specifications and the drawings which relate to

several variations of a preferred embodiment of the present invention.

#### DESCRIPTION OF THE PREFERRED EMBODIMENTS

The manufacturing process of the present invention will be easily understood in broad aspects by reference to FIG. 1a wherein there is illustrated the basic steps in the manufacture of the magnetically permeable ceramic tape. The construction principle of the multi-layer ceramic inductor chip begins with the mixing of a slurry 31 of alumina powder and various binders that can be cast in thin layers 31 on a flat surface 34. However, before casting a magnetically permeable powder 32 is added to the slurry of ceramic material 31. A doctor-blade 33 is normally used to achieve the required thinness and uniformity. Organic binders in the slurry give enough strength and flexibility to the tape 31 after drying for removal and handling. Strips 37 are cut out of this tape and backed with insulating paper 36 and then holes are punched with tool 38 and the resulted strips are rolled onto reels 39. The striping or cutting of strips is done with tool 35. In order that this particular portion of the process may be easily understood it is presented to flow chart form. In FIG. 1b step 40 consists of adding a portion of magnetic powder to the ceramic slurry 31. The proportion of the magnetic material to the ceramic material may vary between 5 and 30 percent of the volume of the ceramic material. The next step of the process 41 is to spread this slurry material by doctor blade to the desired thickness. After step 41 is accomplished the ceramic sheet material is dried, step 42, by convection or infrared or other heat transfer means. Once the ceramic sheet material is dry it acquires a plastic and rubber like characteristic and becomes very flexible, yet not brittle. In step 43, this tape-like, rubber-like material is cut into long strips 37. In order to prevent the slurry tapes from sticking together due to temperature changes during rolling, a paper or plastic backing is apposited, step 44, to the tape and the tape is then in step 45 punched with holes at the required locations. The long strips of tape are next rolled onto reels, step 46. This completes the process for formation of the tape.

The next phase necessary in the production of these monolithic microminiature inductance elements with magnetically permeable ceramic cores is a formation of conductive paths by pattern deposition as shown in FIG. 2a. The reels of ceramic tape 39 are fed through a printer 47 which screens the conductive pattern necessary to form the inductance element onto the tape 37. The tape 37 is then fed through a drying oven or apparatus 49 which removes the highly volatile components of the metalization silk screened onto the substrate 37. After the metalization is dried the paper is separated from the ceramic tape 37 and rolled onto reels 50 for reuse. The ceramic tape 37 is then fed into a compression and lamination apparatus 51 along with reels of tape from other lines similar to the one we have described as illustrated in 52. Sections of these sheets are aligned and stacked and the stacked structure 53 is compressed and laminated by compression apparatus 51 and the resulting compressed structure is cut from the tape sources and trimmed with cutting apparatus 54. These large compressed sheets of ceramic tape with metalization thereon contain many inductors. These laminated structures 56 are then carried by a belt 55 to

a sintering oven 57 which cures the ceramic at temperatures up to 1,600° C. transforming the laminated structure 56 into a monolithic mass of conductor, ceramic, and magnetically permeable powder immersed and surrounded by the various granules and molecules of alumina ceramic. Once this essential step is completed it is necessary to use a diamond cutter 58 to cut out the various conductors comprised in structure 56. The above steps are illustrated in flow chart form in 10 FIG. 2b. Note that in step 66 of FIG. 2b metal terminations are attached to the individual inductive elements. Step 66 is a final increment in the production of these elements. In particular, FIG. 3a shows the various steps necessary in order to form the proper pattern and to get the proper interconnections between the various layers to compose a helical inductor. If we were to take an inductor cut from the laminated 56 which, for instance, is comprised of seven individual layers of tape the structure would look as indicated and illustrated in 15 FIG. 3a.

In order to appreciate the relationship between the various layers in the laminated structure 56, continuing reference is made to FIG. 3a. Reference character A represents a first layer or lamination that has its top side indicated by 207 and its bottom side indicated by 200. The top side 207 has a large rectangular metalization or bonding pad 240 thereon. This pad is used to bond the resulting helical inductor to other circuits. A hole 241 is formed in a corner of the pad 240. The bottom side 200 of the layer A has a small rectangular interconnection pad 220 formed thereon. The hole 241 previously mentioned in connection with the top side 207 is the same hole 241 that passes through the interconnection pad 220. If one were to flip the layer A from the bottom side 200 to the top side 207, by rotating the layer to the left as it is being flipped, the configuration as depicted in FIG. 3a, for the top side 207 will be seen. The supporting tape between the conductive 25 portions 220 and 240 constitutes the ceramic tape previously discussed which is magnetically permeable but electrically insulative.

A similar relationship between top and bottom sides exists for layer B. The layer B has a single, discontinuous loop formed on the bottom side 201. Interconnection pads 221 and 222 are positioned in spaced perpendicular relationship to each other. A hole 243 is formed through the interconnection pad 221. This hole, as well as the previously mentioned hole 241 is formed at 38 30 in FIG. 1a. The top side of the layer B has a single interconnection pad 242 with the hole 243 passing therethrough. Thus, the hole 243 passes through the interconnection pad 242 on the top side as well as the interconnection pad 243 of the loop which is formed on the bottom side of layer B. To visualize the relationship between the top and bottom sides in three dimensions, one must visualize the bottom side 201 being flipped over to the opposite top side, the flipping occurring by turning the layer B over to the left in which case it will be clear that the hole 423 in the top side is positioned in registry with the hole 243 of the bottom side. This relationship between top and bottom sides of the layers in the lamination 56 exists for the upper and lower depicted layers in FIG. 3a. As a result, seven layers are shown. When the layers are arranged in juxtaposition with one another, then the following relationship exists 35 between interconnecting members.

The upper most layer 240 is connected with an underside interconnection pad 220, through a conductor existing in the opening 241. In the present invention, the conductor referred to is actually fused metal that is contributed by the bonding pad 240 on the top side and the interconnection pad 220 on the bottom side. The interconnection pad 220 contacts the interconnection pad 242 of top side 208 in the next lower layer B. Fused metal from the hole 243 forms a conductive path between the pad 242 and the pad 221 on the under side 201. A thin loop or conductor in the form of a generally U-shaped configuration continues the conductive path to the pad 222 at the other end of the loop. Thus far, a conductive path has been formed between the bonding pad 240 and the first turn of the resulting helical inductor laminate inductor 56. Next comes the top side 209 of the next layer. When so situated in the laminated structure, contact is made between the pad 222 of the previously mentioned loop and an interconnection pad 245 in 209. A hole 244 passes through the interconnection pad 245 and a similarly situated interconnection pad 223 on the bottom side of this layer. Fused metal during the compression step causes the interconnection of the pads. A second loop exists on the bottom layer 202 which terminates in another interconnection pad 224 at the opposite end of the loop. Thus, a conductive path has been completed through two windings of the helical inductor. The top side of the next layer lays in juxtaposition with the bottom layer 202 of the layer above it. More specifically, the interconnection pad 224 of side 202 contacts the interconnection pad 246 of top side 210 in the forth layer. A hole 247 is formed through the layer and an interconnection pad 225 on the bottom side 203 of this bottom layer. The interconnection pad 225 is connected to a third loop or winding that terminates outwardly in an interconnection pad 226. Thus far described, a conductive pad has been formed between the bonding pad 240 and the interconnection pad 226 thus completing three windings of the helical inductor. The next lower lamination has its top side 211 positioned against the lower side 203 of the lamination above it. Particularly, the previously mentioned interconnection pad 226 contacts the interconnection pad 248 on the top side 211. A hole 249 passes through the interconnection pad 248 and an interconnection pad 227 on the bottom side 204 of the fifth layer. A conductive loop or winding connects the interconnection pad 227 to the interconnection pad 228 at the opposite end of the winding. The hole 249 again permits the fusing of metal between the interconnection pads 248 and 227 on opposite sides of the layer thus creating a conductive path through the layer. Thus far described, an electrical path has been described between the bonding pad 240 and a fourth winding of the helical inductor.

Continuing with the next lower lamination, the top side 212 of the sixth layer includes an interconnection pad 250 with a hole 251 formed therein. This hole passes through a similarly disposed interconnection pad 229 on the bottom side of the sixth layer. As in other cases, an additional winding is formed on this bottom side. The hole 251 again provides space for fused metal from the interconnection pads 250 and 229 to interconnect these pads through the layer. The interconnection pad 230 at one end of the fifth winding contacts an interconnection pad 252 on the top side of the seventh layer. A hole 253 is formed through the in-

terconnection pad 253. This hole passes through the rectangular metalization or bonding pad 231 which exists on the bottom side of the seventh layer. Due to the presence of this hole, metal fuses between the interconnection pad 252 and the bonding pad 206 to complete an electrical path through the complete helical inductor including the five turns on the bottom sides of the second-sixth layers of the structure.

It is most significant to note that the present invention includes the inventive concept of using an identical configuration on the bottom sides of previously discussed second-sixth layers in FIG. 3a. Further, the same simple interconnection pad exists on the top side of these layers. Thus, by merely using seven identical layers a helix can be formed by rotating each layer or lamination by 90° with respect to the one above it and below it. The top most or first layer A and the last or bottom most layer, which is the right most layer in FIG. 3a, are identical. They only differ in that the top side of the top most layer A is reversed in relationship to the bottom most layer. This type of modular approach expedites the fabrication of the device and results in minimum cost considerations.

Referring now to FIGS. 3b, 3c, 3d and 5b we outline two possible methods for providing terminations for the monolithic inductor. One species comprises one kovar cross-shaped (FIG. 3b) or u-shaped (FIGS. 5b and 5c) sheet attached to each end of the monolithic inductor 67. The kovar metal sheet termination 69 or a sheet made out of a similar metal such as gold or silver or platinum or lead tin is attached to the bonding pad 73 at the end of the inductor either by soldering 69 and binding the tabs around the end of the inductor or welding 69 to the bonding pad 73. Bonding pads 73 and bonding pads 72 can be coated with high temperature solder and then joined. This joining may be accomplished by an electric heating means 70. One way of attaching the terminations 69 formed onto the inductor 67 and thus forming 68 is to use the combination of members 71 and 70 as a high resistance heating element passing current thereinto and thus joining the terminations to the inductor by soldering. Another possibility is to use member 71 as the electrodes of a high resistance weld apparatus and thus weld the end terminations 69 to the attachment pad 73. An alternative process is to dip each end of the monolithic inductor 67 into a thixotropic paste 74 and coat each end thereof as illustrated in 75. The entire structure 75 is then sintered in a high temperature oven. Several compositions of paste 74 are acceptable. Among these are gold, platinum-gold, platinum-silver, copper, palladium-silver, molymanganese, and lead-tin. The final product of this process is so illustrated in FIG. 3e.

On FIG. 4 is shown a flow chart of the manufacturing process by subtractive etching. Summarizing this process, first the tape is coated with a layer of metal. This may be done either by spraying of a thick-film thixotropic paste or by vacuum deposition of a metal by thin-film technique. Both sides of the tape are coated. Next each side of the tape is coated with photoresist. This may be done by spraying or other dipping or bathing means. The photoresist is exposed in a pattern apposited to both sides as illustrated in step 82. Next the photoresist is developed in the proper solution and then the tape is immersed in an etchant to remove the unwanted areas of metal. Upon completion of this step 83

the photoresist is removed from the metallization in step 84.

On step 86 one electrode layer is aligned and juxtaposed to a layer comprising one layer of the inductor. After completion of the previous step 86 the next layer is rotated 90° and aligned and juxtaposed. This step 87 is repeated  $n$  times,  $n$  being proportional to the value of the inductance desired. Finally, the top electrode layer is properly aligned and juxtaposed, step 89. The aligned and juxtaposed layers including the electrode layers are then compressed under pressure. The compressed layers are sintered in a high temperature kiln at temperatures above 1,500° C. The center sections are then cut into single inductors utilizing a diamond saw, step 92. Next, the electrodes are applied to the inductors, step 93. In the final step of manufacture of these inductors the electrodes are either welded onto the pad as shown in step 94, sintered onto the inductor as shown in step 95, or soldered on as shown in step 96.

FIG. 5a provides an exploded view of the monolithic microminiature inductor without end terminations. FIG. 5a also shows the various building blocks necessary to construct a complete inductor. Note that each building block has only one hole for interconnection. 25

Tracing the electrical path from the termination bonding pad 119 is FIG. 5d, the metallization may be followed through hole 114 to the pad 109 in FIG. 5a which is connected to the conductive pad 111. This pad 111 is then connected to inductive pad 109 of the next layer 201. Pad 112 is connected via hole 112 to pad 109. Pad 109 of layer 101 is connected via path 110 through a metallized hole in 102 to conductive pad 113. The conductive pad 113 of layer 102 is connected to pad 109 of layer 103 and then to pad 111 thereon. The conductive pad 111 of layer 103 connects to pad 109 of layer 104 which connects to pad 111 thereon. Pad 111 of layer 104 connects to pad 116 shown in FIG. 5f. Metallized hole 115 interconnects pad 116 of 40 layer 105 with termination bonding pad 120 thereon.

In FIG. 5b the end termination comprising kovar metal is illustrated. This end termination 122 has on its inner central face a solder material 123 for connection and joining to a termination bonding pad 120 or 119. Soldering or welding may be accomplished by applying the appropriate amount of thermal power to the portion 124. In the case of welding, a current is passed through the termination 122 at the point 124. 45

Turning further to FIGS. 6a and 6b the intricacies of interconnecting a metallization pad on the surface of one layer or segment to a metallization pad on the surface of another layer or segment are described. FIG. 6a shows two layers 102 and 103 of ceramic tape with metallizations 109 and 111 thereon and through-hole 112 therein before lamination and interconnection. Ceramic tape 103 is positioned and aligned on top of ceramic tape 102. Apposited onto ceramic tape 102 is a metallization connection pad 111. This metallization connection pad 111 is connected to metallization connection pad 109 through aperture or hole 112. It is 50

noted that hole 112 is metallized throughout. FIG. 6b shows two ceramic tape layers apposited to each other and appropriately compressed. What is shown in ceramic tape 103 on top of and juxtaposed to the ceramic tape 102. Metallized hole 112 is compressed into metallized connection layer and pad 111 forming a continuous conductive path from 111 to pad 109 with the metallization in hole 112 serving as the connecting means.

10 It is to be understood that barium titanate (BaTiO<sub>3</sub>) may also be used in the slurry to enhance the properties of the refractory ceramic.

15 The inventor wishes it to be understood furthermore that he does not desire to be limited to the exact detail of construction shown and described herein for obvious modifications will occur to a person skilled in this art.

What is claimed is:

1. A microminiature inductor in the form of a monolithic ceramic block having apposited layers, each layer comprising:

a member having a body portion made of magnetically permeable and electrically insulative metal powder immersed in said block; a first side of each member having a formation thereon characterized as a discontinuous conductive loop with conductive interconnection pads at the ends thereof;

a second side of each member having a formation thereon characterized as a conductive interconnection pad, the formation on respective sides of each of said members being identical in configuration, one of the interconnection pads on the end of each loop being positioned in registry with the interconnection pad on the opposite side of the member; an opening formed through the interconnection pad on the second side of each member;

the members stacked so that all first sides face in one direction while the second sides face a second direction;

each member being rotated substantially 90° with respect to the member above and below it to cause the interconnection pad on the second side of each member to be in contact with an interconnection pad on the first side of a juxtaposing member;

metal material from contacting interconnection pads fused together through a hole in the interconnection pad of a respective second side thus resulting in a conductive helix formed through the members with the body portions of the members serving as a core for the helix.

2. The subject matter of claim 1 together with two layers having conductive bonding pads thereon, the layers being electrically connected to the helix ends for providing connection terminals to the helix.

3. The subject matter of claim 2 wherein the body of the member comprises an electrically insulated, magnetically permeable metal powder immersed in ceramic, said powder and ceramic forming a contiguous material, whereby said ceramic is made magnetically permeable by the presence of said powder.

\* \* \* \* \*